

## UNITED STATES PATENT OFFICE

ALBERT C. FISCHER, OF CHICAGO, ILLINOIS, ASSIGNOR TO THE PHILIP CAREY MANUFACTURING COMPANY, A CORPORATION OF OHIO

## CONSTRUCTIONAL MATERIAL

No Drawing.

Application filed December 7, 1925. Serial No. 73,928.

The improved construction material is prepared in sheet form and may be utilized for expansion joint purposes, roofing, siding, floor covering, deck covering, individual and 5 strip shingles, and the like.

I have found when a binding material has finely divided fibre added to it, and strips of strengthening material are added thereto in certain proportions, that a very strong sheet 10 can be developed, said binding material is preferably a waterproof material or a waterproof binder, and it may be understood that the binding material may in itself develop great tensile strength, depending largely 15 upon how it is fabricated.

A resin rubber compound filled with fibrous matter will be a much stronger binder than bituminous matter having a paraffine base. Likewise bituminous material having an 20 asphalt base, will be much stronger than the bituminous material having a paraffine base. Likewise an asphaltic binder produced from Mid Continent residues or Mexican residues, which are more tenacious.

25 Considerable variations may be experienced in the waterproof binder, and for the purpose of this invention I will give the preferred formula of asphaltic material having a penetration on a Howard V. Morse, N. Y. 30 Testing Laboratories, pentrometer of from 21 to 25 degrees at 32° F., 25 to 30 degrees at 77° F. and 35 to 45 degrees at 115° F., the melting point ranging from 220° to 260°. This particular binding material is soluble 35 in carbondisulphide to the extent of 99.6 per cent.

By adding to this binding material uncoagulated latex or by adding to this binding material dissolved rubber it can be greatly 40 strengthened, but likewise the expense will greatly increase. Therefore, I prefer the formula outlined as the binder.

I find that finely divided fibrous material 45 distributed thru said binder also aids in strengthening it, and adds toughness thereto, said finely divided material may be such materials as cotton, jute fibre, wood pulp, linters, roofing scrap, which also has some asphaltic 50 matter distributed therethru, or in fact any

finely divided fibrous material which will add bulk.

I find that said proportions of fibre may range from fifteen (15) to fifty (50) per cent, and that when incorporated in the binder it 55 adds a bulk strengthening material. The preferred fibrous matter which I utilize in this formula consists of roofing scrap, in which the finely divided fibres are intermingled with bituminous material and coated 60 therewith, and for my preferred formula I incorporate forty (40) per cent of this material with fifty-one (51) per cent of the formula noted for the binder.

My range of percentages for the binder is 65 from forty-five (45) to sixty-three (63) per cent, this range producing the best result, and as stated, other binders toughened at greater expense may be more effective, but for the purpose of this invention the preferred form of 70 fifty-one (51) per cent asphalt, of the type described, and forty (40) per cent roofing scrap, of the type described, will answer the purpose.

As a strengthening material I employ corn 75 husks, tough grasses, or in fact any vegetation or web which is flat, as distinguished from round, and has considerable strong fibre in the web state.

My preferred formula is to utilize corn 80 husks dry, of which materials I use nine (9) per cent. The percentages of husk materials range from five (5) per cent to seventeen (17) per cent, but I find that nine (9) per cent of this particular strengthening web together 85 with forty (40) per cent of the roofing scrap and fifty-one (51) per cent of the asphalt described give the best results. Alternating proportions of these same materials, where a lesser percentage of husks and a greater 90 percentage of roofing chips is shown show a weaker structure. Likewise, where a higher percentage of strengthening web and a lower percentage of roofing chips are employed together with a higher percentage of asphalt, 95 I find that the tensile strength decreases.

A paraffin base, blown asphalt, will show a tensile strength of approximately forty (40) pounds to the square inch. An asphalt 100 containing a Mexican asphalt can be pre-

pared to show a tensile strength of sixty (60) pounds to the square inch.

The strongest expansion joint, previous to this invention, shows a tensile strength of 240 lbs. to the square inch, and the formula outlined herein gives a material having a tensile strength of 313 pounds to the square inch at a room temperature of 70 degrees, at which these tests were made.

10 To better illustrate the characters of my improved construction material I disclose a tabulation of the approximate tensile strengths in pounds per square inch, obtained by varying the amounts of the materials entering into the formation of the construction material.

| 20 | Bitumi-        | Asphalt  | Husks    | Tensile       |
|----|----------------|----------|----------|---------------|
|    | nous<br>fibers | Per cent | Per cent | strength #/□" |
| 25 | 45             | 50       | 5        | 301           |
|    | 48             | 45       | 7        | 309           |
|    | 51             | 40       | 9        | 313           |
|    | 54             | 35       | 11       | 296           |
|    | 57             | 30       | 13       | 291           |
|    | 60             | 25       | 15       | 260           |
|    | 63             | 20       | 17       | 254           |

From this table it will be noted that the maximum strength disclosed is obtained when the mixture comprises fifty-one (51) per cent fibrous material mixed with bitumen, forty (40) per cent asphalt and nine (9) per cent husk material. By decreasing or increasing the husk content the tensile strength is lowered.

35 The materials are suitably mixed in a power mixer, placed between pressing rolls, rolled into sheets and cut into strips. I find that it is not advantageous to mix too long, as it is detrimental to break the fibre in exceedingly small pieces. The strength of the material will be in proportion to the size at which the strengthening web material can be incorporated, but the strength herein lies in the bulk rather than in a mass covered with an outer web of reinforcing means.

40 It is preferred that flat, strengthening webs be employed rather than rounded fibres, such as, broom corn, straw, and the like, as the flat particles spread themselves over the mastic area and thus add rigidity to the mass. After being pressed into shape these strengthening webs form themselves into interlaced or staggered relation, running lengthwise of the sheet, and flattening themselves pretty much over given areas. The sheet so prepared may then be employed for structural materials of various kinds, as cited, and this material is particularly adapted for expansion joint purposes because of the tensile strength at elevated temperatures.

45 I claim:

1. Preformed constructional material composed of a plastic mass containing a ductile waterproofing binder, finely divided

roofing scrap, and reenforcing elements of relatively large surface areas.

2. Preformed constructional material composed of a plastic mass containing a ductile waterproofing binder, finely divided roofing scrap and corn husks. 70

3. Preformed constructional material composed of a plastic mass containing a ductile waterproofing binder, finely divided roofing scrap, rubber, and reenforcing elements of relatively large surface areas. 75

4. Preformed constructional material composed of a plastic mass containing a predominating proportion of ductile waterproofing binder and a subordinate proportion of finely divided roofing scrap and reenforcing elements of relatively large surface areas. 80

5. Preformed expansion joint strips composed of a plastic mass containing a ductile waterproofing binder, finely divided roofing scrap, and reenforcing elements of relatively large surface areas. 85

6. Preformed expansion joint strips composed of a plastic mass containing a ductile waterproofing binder, finely divided roofing scrap and corn husks. 90

7. Preformed expansion joint strips composed of a plastic mass containing a ductile waterproofing binder, finely divided roofing scrap, rubber, and reenforcing elements of relatively large surface areas. 95

8. Preformed expansion joint strips composed of a plastic mass containing a predominating proportion of ductile waterproofing binder and a subordinate proportion of finely divided roofing scrap and reenforcing elements of relatively large surface areas. 100

9. A composition of matter composed of a plastic mass containing a ductile waterproofing binder, finely divided roofing scrap, and reenforcing elements of relatively large surface areas. 105

10. A composition of matter composed of a plastic mass containing a ductile waterproofing binder, finely divided roofing scrap and corn husks. 110

11. A composition of matter composed of a plastic mass containing a ductile waterproofing binder, finely divided roofing scrap, rubber, and reenforcing elements of relatively large surface areas. 115

12. A composition of matter composed of a plastic mass containing a predominating proportion of ductile waterproofing binder and a subordinate proportion of finely divided roofing scrap and reenforcing elements of relatively large surface areas. 120

Signed at Chicago, Illinois this 4th day of Dec., 1925. 125

ALBERT C. FISCHER.